

## UNITED STATES PATENT OFFICE.

EDGAR F. PRICE, OF NIAGARA FALLS, NEW YORK, ASSIGNOR TO UNION CARBIDE COMPANY, OF NIAGARA FALLS, NEW YORK, A CORPORATION OF VIRGINIA.

## ELECTRODE.

SPECIFICATION forming part of Letters Patent No. 779,783, dated January 10, 1905.

Application filed June 28, 1904. Serial No. 214,452.

*To all whom it may concern:*

Be it known that I, EDGAR F. PRICE, a citizen of the United States, residing at Niagara Falls, in the county of Niagara and State of New York, have invented certain new and useful Improvements in Electrodes, of which the following is a specification.

United States Patent No. 757,036, granted April 12, 1904, to John J. Griffin, describes a process of producing chemical compounds by electrolyzing solutions with an electrode of a metallic carbide which will react chemically on the electrolyte, especially one of calcium carbide. It is difficult, however, to obtain pieces of calcium carbide of sufficient size, regular shape, and uniform composition to serve as practical electrodes, and the reaction between the carbide and aqueous solutions is apt to disintegrate and destroy the electrode.

The present invention is a composite electrode of a carbide and a binder, the preferred binding agent being a coked hydrocarbon or carbonaceous substance, such as bituminous coal.

To produce these composite electrodes, the carbide—for example, calcium carbide—is crushed and mixed with the binding agent—for example, five to twenty-five per cent., by weight, of pulverized bituminous coal and a small amount of water-free tar or pitch. The mixture is then molded into the desired form by a press or by forcing it through a die and cutting the product into lengths. The molded pieces are then baked at a temperature sufficiently high to decompose the hydrocarbons and drive off the volatile matter, converting the bituminous coal and tar into coke. This coke not only binds the particles of carbide into a hard coherent body, but increases the

electrical conductivity, and is especially useful when the electrodes are employed in aqueous solutions, as it retards the action of the water upon the carbide, although its porosity permits the water to finally react on all of the carbide. The porosity of the electrode may be decreased, if desired, by saturating it with a liquid hydrocarbon or carbohydrate and again baking it, thereby depositing more carbon in the pores.

The upper end of the electrode may be filled with paraffin and provided with any approved terminal, such as a body of antimonial lead cast around it.

I claim—

1. An electrode, comprising a carbide and a binder, as set forth.
2. An electrode, comprising a carbide and a carbon binder, as set forth.
3. An electrode, comprising a carbide and a coked binder, as set forth.
4. An electrode, comprising calcium carbide and a binder, as set forth.
5. An electrode, comprising calcium carbide and a carbon binder, as set forth.
6. An electrode, comprising calcium carbide and a coked binder, as set forth.
7. An electrode, comprising calcium carbide and a binder containing coked bituminous coal, as set forth.
8. An electrode, comprising calcium carbide and a binder of coked bituminous coal and a liquid hydrocarbon, as set forth.

In testimony whereof I affix my signature in presence of two witnesses.

EDGAR F. PRICE.

Witnesses:

WILLIAM SMITH HARRY,  
GEO. H. DANFORTH.